# EUROPEAN PATENT SPECIFICATION

(11) **EP 1 600 515 B1**
(45) Date of publication and mention of the grant of the patent: **30.07.2008**
(21) Application number: 05017189.1
(22) Date of filing: 16.11.1998
(51) Int. Cl.: C22C 9/04, C22F 1/08

(54) **Lead-free, free-cutting copper alloys**
Bleifreie Automatenkupferlegierung
Alliage de cuivre de décolletage sans plomb

(30) Priority: 12.10.1998 JP 28859098
(43) Date of publication of application: 30.11.2005
(62) Divisional of application: 98953071.2
(73) Proprietor: Sambo Copper Alloy Co., Ltd, Osaka 590-0906 (JP)
(72) Inventor: Oishi, Keiichiro, Sakai-shi Osaka 590-0906 (JP)
(74) Representative: Rees, Kerry

(56) References cited:
- FR-A- 1 031 211
- US-A- 2 237 774
- PATENT ABSTRACTS OF JAPAN vol. 1998, no. 04, 31 March 1998 (1998-03-31) -& JP 09 316570 A (CHUETSU GOKIN CHUKO KK), 9 December 1997 (1997-12-09)
- PATENT ABSTRACTS OF JAPAN vol. 015, no. 227 (C-0839), 10 June 1991 (1991-06-10) -& JP 03 068731 A (NIPPON MINING CO LTD), 25 March 1991 (1991-03-25)
- PATENT ABSTRACTS OF JAPAN vol. 1997, no. 10, 31 October 1997 (1997-10-31) -& JP 09 143598 A (CHUETSU GOKIN CHUKO KK), 3 June 1997 (1997-06-03)

## Description

### BACKGROUND OF THE INVENTION

### 1. Field of The Invention

The present invention relates to lead-free, free-cutting copper alloys.

### 2. Prior Art

Among the copper alloys with a good machinability are bronze alloys such an the one under JIS designation H5111 BC6 and brass alloys such an the ones under JIS designations H3250-C3604 and C3771. Those alloys are enhanced in machinability by the addition of 1.0 to 6.0 percent, by weight, of lead and provide an industrially satisfactory machinability. Because of their excellent machinability, those lead-contained copper alloys have been an important basic material for a variety of articles such as city water faucets, water supply/drainage metal fittings and valves.

However, the application of those lead-mixed alloys has been greatly limited in recent years, because lead contained therein is an environment pollutant harmful to humans. That is, the lead-containing alloys pose a threat to human health and environmental hygiene because lead is contained in metallic vapor that is generated in the steps of processing those alloys at high temperatures such as melting and casting and there is also concern that the lead contained in the water system metal fittings, valves and others made of those alloys will dissolve out into drinking water.

On that ground, the United States and other advanced countries have been moving to tighten the standards for lead-contained copper alloys to drastically limit the permissible level of lead in copper alloys in recent years. In Japan, too, the use of lead-contained alloys has been increasingly restricted, and there has been a growing call for development of free-cutting copper alloys with a low lead content.

JP-A-9-316570 discloses an end bearing for a one way clutch having high wear resistance having manganese silicide type high strength brass having ≤30% beta phase in its metallic structure. The brass has a chemical composition comprising (1) by weight 15-37% Zn, 0.3-5.0% Mn, 0.3-3.0% Si, and the balance Cu. In addition the composition may composition one or more elements selected from the group consisting of 0.1-5% Al, 0.1-4% Ni, Co, Pb or Bi, 0.1-3% Sn or Fe, 0.05-2% Cr, Ti, V, Zr, Nb or Mo.

### SUMMARY OF THE INVENTION

It is an object of the present invention to provide a lead-free copper alloy which does not contain the machinablility-improving element lead yet is quite excellent in machinability and can be used as safe substitute for the conventional free cutting copper alloy with a large content of lead presenting environmental hygienic problems and which permits recycling of chips without problems, thus a timely answer to the mounting call for restriction of lead-contained products.

It is another object of the present invention to provide a lead-free copper alloy which has a high corrosion resistance as well as an excellent machinability and is suitable as basic material for cutting works, forgings, castings and others, thus having a very high practical value. The cutting works, forgings, castings and others include city water faucets, water supply/drainage metal fittings, valves, stems, hot water supply pipe fittings, shaft and heat exchanger parts.

It is yet another object of the present invention to provide a lead-free copper alloy with a high strength and wear resistance as well as machinability which is suitable as basic material for the manufacture of cutting works, forgings, castings and other uses requiring a high strength and wear resistance such as, for example, bearings, bolts, nuts, bushes, gears, sewing machine parts and hydraulic system parts, hence has a very high practical value.

It is a further object of the present invention to provide a lead-free copper alloy with an excellent high-temperature oxidation resistance as well as machinability which is suitable as basic material for the manufacture of cutting works, forgings, castings and other uses where a high thermal oxidation resistance is essential, e.g. nozzles for kerosene oil and gas heaters, burner heads and gas nozzles for hot-water dispensers, hence has a very high practical value.

The objects of the present inventions are achieved by provision of the following copper alloy:
The present invention provides a lead-free free-cutting copper alloy also with an excellent machinability and with an excellent high strength feature and high corrosion resistance which is composed of 62 to 78 percent, by weight, of copper; 2.5 to 4.5 percent, by weight, of silicon; at least one element selected from among 0.3 to 3.0 percent, by weight, of tin, 0.2 to 2.5 percent, by weight, of aluminium, and 0.02 to 0.25 percent, by weight, of phosphorus; at least one element selected from among 0.7 to 3.5 percent, by weight, of manganese and 0.7 to 3.5 percent, by weight, of nickel; optionally at least one element selected from among 0.02 to 0.4 percent, by weight, of bismuth, 0.02 to 0.4 percent, by weight, of tellurium, and 0.02 to 0.4 percent, by weight, of selenium; and the remaining percent, by weight, of zinc.
The present invention also provides a method of forming a lead-free, free cutting alloy which comprises having a metal structure which has at least one phase selected from the γ (gamma) phase and the κ (kappa) phase which comprises alloying copper and silicon in an amount of 62 to 78 percent, by weight, of copper; 2.5 to 4.5 percent, by weight, of silicon; at least one element selected from tin, aluminium and phosphorous in an amount of 0.3 to 3.0 percent, by weight, of tin, 0.2 to 2.5 percent, by weight, of aluminium and 0.02 to 0.25 percent, by weight, of phosphorous; at least one element selected from manganese and nickel in an amount of 0.7 to 3.5 percent, by weight, of manganese and 0.7 to 3.5 percent, by weight, of nickel; optionally at least one element selected from bismuth, tellurium and selenium in an amount of 0.02 to 0.4 percent, by weight, of bismuth, 0.02 to 0.4 percent, by weight, of tellurium and 0.02 to 0.4 percent, by weight, of selenium; and the remaining percent, by weight, of zinc.
Manganese and nickel combine with silicon to form intermetallic compounds represented by MnxSiy or NixSiy which are evenly precipitated in the matrix, thereby raising the wear resistance and strength. Therefore, the addition of manganese and/or nickel would improve the high strength feature and wear resistance. Such effects will be exhibited if manganese and nickel are added in an amount not smaller than 0.7 percent by weight respectively. But the saturation state is reached at 3.5 percent by weight, and even if the addition is increased beyond that, no proportional results will be obtained. The addition of silicon is set at 2.5 to 4.5 percent by weight to match the addition of manganese or nickel, taking into consideration the consumption to form intermetallic compounds with those elements.

It is also noted that tin, aluminum and phosphorus help to reinforce the alpha phase in the matrix, thereby improving strength, wear resistance, and also machinability. Tin and phosphorus disperse the alpha and gamma phases, by which the strength, wear resistance and also machinability are improved. Tin in an amount of 0.3 or more percent by weight is effective in improving the strength and machinability. But if the addition exceeds 3.0 percent by weight, the ductility will fall. For this reason, the addition of tin is set at 0.3 to 3.0 percent by weight to raise the high strength feature and wear resistance in the alloy of the present invention to enhance the machinability. Aluminium also contributes to improving the wear resistance and exhibits its effect of reinforcing the matrix when added in 0.2 or more percent by weight. But if the addition exceeds 2.5 percent by weight, there will be a fall in ductility. Therefore, the addition of aluminium is set at 0.2 to 2.5 in consideration of improvement of machinability. Also, the addition of phosphorus disperses the gamma phase and at the same time refines the crystal grains in the alpha phase in the matrix, thereby improving the hot workability and also the strength and wear resistance. Furthermore, it is very effective in improving the flow of molten metal in casting. Such results will be produced when phosphorus is added in the range of 0.02 to 0.25 percent by weight. The content of copper is set at 62 to 78 percent by weight in the light of the addition of silicon and bonding of silicon with manganese and nickel.

The alloy of the present invention contains at least one element selected from among 0.02 to 0.4 percent, by weight, of bismuth, 0.02 to 0.4 percent, by weight, of tellurium, and 0.02 to 0.4 percent, by weight, of selenium. Addition of these elements causes an improvement in machinability by adding at least one element selected among bismuth and other elements which are effective in raising the machinability through a mechanism different from that exhibited by silicon.

Bismuth, tellurium and selenium as well as lead do not form a solid solution in the matrix but disperse in granular form to enhance the machinability and that through a mechanism different from that of silicon. Hence, the addition of those elements along with silicon could further improve the machinability beyond the level obtained by the addition of silicon alone. From this finding, the alloy of the present invention is provided in which at least one element selected from bismuth, tellurium and selenium is mixed to improve further the machinability of the alloy of the present invention. The addition of bismuth, tellurium or selenium in addition to silicon produces a high machinability such that complicated forms could be freely cut at a high speed. But no improvement in machinability can be realized from the addition of bismuth, tellurium or selenium in an amount less than 0.02 percent, by weight. Meanwhile, those elements are expensive as compared with copper. Even if the addition exceeds 0.4 percent by weight, the proportional improvement in machinability is so small that the addition beyond that does not pay economically. What is more, if the addition is more than 0.4 percent by weight, the alloy will deteriorate in hot workability such as forgeability and cold workability such as ductility. While it might be feared that heavy metals like bismuth would cause problems similar to those of lead, an addition in a very small amount of less than 0.4 percent by weight is negligible and would present no particular problems. From those considerations, the second invention alloy is prepared with the addition of bismuth, tellurium or selenium kept to 0.02 to 0.4 percent by weight. The addition of those elements, would not effect the proper contents of copper and silicon.

The alloy of the present invention may have further improved machinability obtained by subjecting it to a heat treatment for 30 minutes to 5 hours at 400°C to 600°C.

The alloys of the present invention contain machinability improving elements such as silicon and have an excellent machinability because of the addition of such elements. Of the invention alloys, the alloys with a high copper content which have great amounts of other phases, mainly kappa phase, than alpha, beta, gamma and delta phases can further improve in machinability in a heat treatment. In the heat treatment, the kappa phase turns to a gamma phase. The gamma phase finely disperses and precipitates to further enhance the machinability. The alloys with a high content of copper are high in ductility of the matrix and low in absolute quantity of gamma phase, and therefore are excellent in cold workability. But in case cold working such as caulking and cutting are required, the aforesaid heat treatment is very useful. In other words, among the alloys of the present invention, those which are high in copper content with gamma phase in small quantities and kappa phase in large quantities (hereinafter referred to as the "high copper content alloy") undergo a change in phase from the kappa phase to the gamma phase in a heat treatment. As a result, the gamma phase is finely dispersed and precipitated, and the machinability is improved. In the manufacturing process of castings, expanded metals and hot forgings in practice, the materials are often force-air-cooled or water cooled depending on the forging conditions, productivity after hot working (hot extrusion, hot forging etc.), working environment and other factors. In such cases, among the alloys of the present invention, those with low content of copper (hereinafter called the low copper content alloy") are rather low in the content of the gamma phase and contain beta phase. In a heat treatment, the beta phase changes into gamma phase, and the gamma phase is finely dispersed and precipitated, whereby the machinability is improved. Experiments showed that heat treatment is especially effective with high copper content alloys where mixing ratio of copper and silicon to other added elements (except for zinc) A is given as 67 ≤ Cu - 3Si + aA or low copper content alloys with such a composition with 64 ≥ Cu - 3Si + aA. It is noted that a is a coefficient. The coefficient is different depending on the added element A. For example, with tin a is - 0.5; aluminium, -2; phosphorus, -3; antinomy, 0; arsenic, 0; manganese, +2.5; and nickel, +2.5.

But a heat treatment temperature at less than 400°C is not economical and practical, because the aforesaid phase change will proceed slowly and much time will be needed. At temperatures over 600°C, on the other hand, the kappa phase will grow or the beta phase will appear, bringing about no improvement in machinability. From the practical viewpoint, therefore, it is desired to perform the heat treatment for 30 minutes to 5 hours at 400 to 600°C.

### BRIEF DESCRIPTION OF THE DRAWING

Fig. 1 shows perspective views of cuttings formed in cutting a round bar of copper alloy by lathe.

### DETAILED DESCRIPTION OF THE PREFERRED EMBODIMENTS

### Example 1

As the first series of examples of the present invention, cylindrical ingots with compositions given in Tables 1 to 18, each 100 mm in outside diameter and 150 mm in length, were hot extruded into a round bar 15 mm in outside diameter at 750°C to produce the following test pieces: alloys Nos. 7001 to 7030 and 8001 to 8147.

As comparative examples, cylindrical ingots with the compositions as shown in Table 19, each 100 mm in outside diameter and 150 mm in length, were hot extruded into a round bar 15 mm in outside diameter at 750°C to obtain the following round extruded test pieces: Nos. 14001 to 14006 (hereinafter referred to as the "conventional alloys"). No. 14001 corresponds to the alloy "JIS C 3604", No. 14002 to the alloy "CDA C 36000", No. 14003 to the alloy "JIS C 3771", and No. 14004 to the alloy "CDA C 69800", No. 14005 corresponds to the alloy "JIS C 6191". This aluminium bronze is the most excellent of the expanded copper alloys under the JIS designations with regard to strength and wear resistance. No. 14006 corresponds to the naval brass alloy "JIS C 4622" and is the most excellent of the expanded copper alloys under the JIS designations with regard to corrosion resistance.

To study the machinability of the alloys of the present invention alloys in comparison with the conventional alloys, cutting tests were carried out. In the tests, evaluations were made on the basis of cutting force; condition of chips cut surface condition.

The tests were conducted this ways: The extruded test pieces obtained, as mentioned above, were cut on the circumferential surface by a lathe mounted with a point noise straight tool at a rake angle of - 8 degrees and at a cutting rate of 50 meters/minute, a cutting depth of 1.5 mm, a feed of 0.11 mm/rev. Signals from a three-component dynamometer mounted on the tool were converted into electric voltage signals and recorded on a recorder. From the signals were then calculated the cutting resistance. It is noted that while, to be perfectly exact, an amount of the cutting resistance should be judged by three component forces - cutting force, feed force and thrust force, the judgement was made on the basis of the cutting force (N) of the three component forces in the present example. The results are shown in Table 20 to Table 29.

Furthermore, the chips from the cutting work were examined and classified into four forms (A) to (D) as shown in Fig. 1. The results are enumerated in Table 20 to Table 29. In this regard, the chips in the form of a spiral with three or more windings as (D) in Fig. 1 are difficult to process, that is, recover or recycle, and could cause trouble in cutting work as, for example, getting tangled with the tool and damaging the cut metal surface. Chips in the form of an arc with a half winding to a spiral with two about windings as shown in (C), Fig. 1 do not cause such serous trouble as the chips in the form of a spiral with three or more windings yet are not easy to remove and could get tangled with the tool or damage the cut metal surface. In contrast, chips in the form of a fine needle as (A) in Fig. 1 or in the form of an arc as (B) will not present such problems as mentioned above and are not bulky as the chips in (C) and (D) and easy to process. But fine chips as (A) still could creep into the sliding surfaces of a machine tool such as a lathe and cause mechanical trouble, or could be dangerous because they could stick into the worker's finger, eye or other body parts. Those taken into account, it is appropriate to consider that the chips in (B) are the best, and the second best are the chips in (A). Those in (C) and (D) are not good. In Table 20 to Table 29, the chips judged to be shown in (B), (A), (C) and (D) are indicated by the symbols "●", "○", "Δ" and "×" respectively.

In addition, the surface condition of the cut metal surface was checked after cutting work. The results are shown in Table 20 to Table 29. In this regard, the commonly used basis for indication of the surface roughness is the maximum roughness (Rmax). While requirements are different depending on the application field of brass articles, the alloys with Rmax < 10 microns are generally considered excellent in machinability. The alloys with 10 microns ≤ Rmax < 15 microns are judged as industrially acceptable, while those with Rmax ≥ 15 microns are taken as poor in machinability. In Table 20 to Table 29, the alloys with Rmax < 10 microns are marked "o", those with 10 microns ≤ Rmax < 15 microns are indicated as "Δ" and those with Rmax ≥15 microns are represented by symbol "x".

As is evident from the results of the cutting tests shown in Table 20 to Table 29, the following invention alloys are all equal to the conventional lead- contained alloys Nos 14001 to 14003 in machinability: alloy Nos. 7001 to 7030 and 8001 to 8147. Especially with regard to formation of the chips, those invention alloys are favourably compared not only with the conventional alloys Nos. 14004 to 14006 with a lead content of not higher than 0.1 percent by weight but also Nos. 14001 to 14003 which contain large quantities of lead.

In another series of tests, the alloys of the present invention were examined in comparison with the conventional alloys in hot workability and mechanical properties. For the purpose, hot compression and tensile tests were conducted the following way.

First, two test pieces, first and second test pieces, in the same shape 15 mm in outside diameter and 25 mm in length were cut out of each extruded test piece obtained as described above. In the hot compression tests, the first test piece was held for 30 minutes at 700°C, and then compressed 70 percent in the direction of axis to reduce the length from 25 mm to 7.5 mm. The surface condition after the compression (700°C deformability) was visually evaluated. The results are given in Table 20 to Table 29. The evaluation of deformability was made by visually checking for cracks on the side of the test piece. In Table 20 to Table 29, the test pieces with no cracks found are marked "o", those with small cracks are indicated in "Δ" and those with large cracks are represented by a symbol "x".

The second test pieces were put to a tensile test by the commonly practised test method to determine the tensile strength, N/mm² and elongation, %.

As the test results of the hot compression and tensile tests in Table 20 to Table 29 indicate, it was confirmed that the alloys of the present invention are equal to or superior to the conventional alloys Nos. 14001 to 14004 and No. 14006 in hot workability and mechanical properties and are suitable for industrial use. The alloys of the present invention in particular have the same level of mechanical properties as the conventional alloy No. 14005, the aluminium bronze which is the most excellent in strength of the expanded copper alloys under the JIS designations, and thus have understandably a prominent high strength feature.

### Example 2

As the second series of examples of the present invention, cylindrical ingots with compositions given in Tables 1-18, each 100 mm in outside diameter and 200 mm in length, were hot extruded into a round bar 35 mm in outside diameter at 700°C to produce the following test pieces: alloy Nos. 7001a to 7030a and alloys Nos. 8001a to 8147a. In parallel, cylindrical ingots with compositions given in Table 19 each 100 mm in outside diameter and 200 mm in length, were hot extruded into a round bar 35 mm in outside diameter at 700 C to produce the following alloy test pieces: Nos. 14001a to 14006a as second comparative examples (hereinafter referred to as the "conventional alloys'). It is noted that the alloys Nos. 7001a to 7030a, Nos. 8001a to 8147a and Nos. 14001a to 14006a are identical in composition with the aforesaid copper alloys Nos. 7001 to 7030, Nos. 8001 to 8147 and Nos. 14001 to No. 14006 respectively.

Those alloys Nos. 7001a to 7030a and alloys Nos. 8001a to 8147a were put to wear resistance tests in comparison with the conventional alloys Nos. 14001a to 14006a.

The tests were carried out in this procedure. Each extruded test piece thus obtained was cut on the circumferential surface, holed and cut down into a ringshaped test piece 32 mm in outside diameter and 10 mm in thickness (that is, the length in the axial direction). The test piece was then fitted around a free-rotating shaft, and a roll 48 mm in outside diameter placed in parallel with the axis of the shaft was urged against the test piece under a load of 50 kg. The roll was made of stainless steel under the JIS designation SUS 304. Then, the SUS 304 roll and the test piece put in rotational sliding contact with the roll were rotated at the same rate of revolutions/minute - 209 r.p.m., with multipurpose gear oil being dropped onto the circumferential surface of the test piece. When the number of revolutions reached 100,000, the SUS 304 roll and the test piece were stopped, and the weight difference between the start and the end of rotation, that is, the loss of weight by wear, mg, was determined. It can be said that the alloys which are smaller in the loss of weight by wear are higher in wear resistance. The results are given in Tables 30 to 40.

As is clear from the wear resistance test results shown in Tables 30 to 40, the tests showed that those alloys Nos. 7001a to 7030a and eighth Nos. 8001a to 8147a were excellent in wear resistance as compared with not only the conventional alloys Nos. 14001a to 14004a and 14006a but also No. 14005a, which is an aluminium bronze having a highest wear resistance of the expanded copper alloys under the JIS designations. From comprehensive considerations of the test results including the tensile test results, it may safely be said that the seventh and eighth invention alloys are excellent in machinability and also possess a higher strength feature and wear resistance than the aluminum bronze which is the highest in wear resistance of all the expanded copper alloys under the JIS designations.

**Table 1**

| No. | alloy composition (wt%) | | | | | | | |
|---|---|---|---|---|---|---|---|---|
| | Cu | Si | Sn | Al | P | Mn | Ni | Zn |
| 7001 | 62.9 | 2.7 | 2.6 | | | 2.2 | | remainder |
| 7001a | | | | | | | | |
| 7002 | 64.8 | 3.4 | 1. 8 | | | | 3.1 | remainder |
| 7002a | | | | | | | | |
| 7003 | 68.2 | 4.1 | 0.6 | | | 1.9 | 1.5 | remainder |
| 7003a | | | | | | | | |
| 7004 | 66.5 | 3.5 | 1.9 | 0.9 | | 1.9 | | remainder |
| 7004a | | | | | | | | |
| 7005 | 71.3 | 3.7 | 0.4 | 1.8 | | | 2.3 | remainder |
| 7005a | | | | | | | | |
| 7006 | 73.6 | 2.9 | 0.7 | 2.1 | | 1.3 | 0.8 | remainder |
| 7006a | | | | | | | | |
| 7007 | 70.1 | 3.2 | 0.5 | 1.4 | 0.11 | 1.8 | | remainder |
| 7007a | | | | | | | | |
| 7008 | 77.1 | 4.2 | 0.8 | 2.3 | 0.03 | | 1.8 | remainder |
| 7008a | | | | | | | | |
| 7009 | 67.3 | 3.7 | 2.6 | 0.2 | 0.08 | 0.9 | 1.8 | remainder |
| 7009a | | | | | | | | |
| 7010 | 75.5 | 3.9 | | 2.3 | | 0.8 | | remainder |
| 7010a | | | | | | | | |

**Table 2**

| No. | alloy composition (wt%) | | | | | | | |
|---|---|---|---|---|---|---|---|---|
| | Cu | Si | Sn | Al P | | Mn | Ni | Zn |
| 7011 | 69.8 | 3.4 | | 0.3 | | | 1.3 | remainder |
| 7011a | | | | | | | | |
| 7012 | 71. 2 | 4.0 | | 1.4 | | 2.1 | 1.2 | remainder |
| 7012a | | | | | | | | |
| 7013 | 73.3 | 3.9 | | 2.0 | 0.03 | 3.2 | | remainder |
| 7013a | | | | | | | | |
| 7014 | 65.9 | 2.9 | | 0.3 | 0.21 | | 1.3 | remainder |
| 7014a | | | | | | | | |
| 7015 | 68.8 | 3.9 | | 1.1 | 0.05 | 0.9 | 2.0 | remainder |
| 7015a | | | | | | | | |
| 7016 | 68.1 | 4.0 | 0.4 | | 0.04 | 2.8 | | remainder |
| 7016a | | | | | | | | |
| 7017 | 63.8 | 2.6 | 2.7 | | 0.19 | | 0.9 | remainder |
| 7017a | | | | | | | | |
| 7018 | 66.7 | 3.4 | 1.3 | | 0.07 | 1.2 | 0.8 | remainder |
| 7018a | | | | | | | | |
| 7019 | 67.2 | 3. 6 | | | 0.21 | 1.9 | | remainder |
| 7019a | | | | | | | | |
| 7020 | 69.1 | 3.8 | | | 0.06 | | 2.2 | remainder |
| 7020a | | | | | | | | |

**Table 3**

| No. | alloy composition (wt%) | | | | | | | |
|---|---|---|---|---|---|---|---|---|
| | Cu | Si | Sn | Al | P | Mn | Ni | Zn |
| 7021 | 72.1 | 4.3 | | | 0.07 | 2. 0 | 0.8 | remainder |
| 7021a | | | | | | | | |
| 7022 | 71.3 | 3.9 | | 1.1 | | 3.1 | | remainder |
| 7022a | | | | | | | | |
| 7023a | 70.5 | 3.5 | | 1. 6 | | 2.3 | | remainder |
| 7023a | | | | | | | | |
| 7024 | 70.0 | 3.6 | | 1.5 | | | 3.2 | remainder |
| 7024a | | | | | | | | |
| 7025 | 69.3 | 2.7 | | 2.1 | | 0.9 | | remainder |
| 7025a | | | | | | | | |
| 7026 | 70.2 | 3.5 | | 1.4 | | | 2.1 | remainder |
| 7026a | | | | | | | | |
| 7027 | 65.0 | 2.8 | 2.6 | 2.3 | | 0.8 | | remainder |
| 7027a | | | | | | | | |
| 7028 | 69. 8 | 3.6 | 1.5 | 1.7 | | 2.4 | | remainder |
| 7028a | | | | | | | | |
| 7029 | 71.0 | 3.6 | 0.4 | 0.3 | | 2.2 | | remainder |
| 7029a | | | | | | | | |
| 7030 | 68.4 | 4.2 | 2.6 | | | 3.3 | | remainder |
| 7030a | | | | | | | | |

**Table 4**

| No. | alloy composition (wt%) | | | | | | | | |
|---|---|---|---|---|---|---|---|---|---|
| | Cu | Si | Sn | Al | Bi | Te | Se | Mn | Zn |
| 8001 | 62.6 | 2.6 | 2.6 | | 0.31 | | | 1.9 | remainder |
| 8001a | | | | | | | | | |
| 8002 | 65.3 | 3.4 | 1.8 | | 0.11 | 0.02 | | 2.5 | remainder |
| 8002a | | | | | | | | | |
| 8003 | 66.4 | 4. 2 | 0.5 | | 0.05 | | 0.03 | 3.4 | remainder |
| 8003a | | | | | | | | | |
| 8004 | 72.1 | 4.4 | 0.4 | | 0.06 | 0.05 | 0.02 | 2.8 | remainder |
| 8004a | | | | | | | | | |
| 8005 | 67.4 | 3.3 | 2.3 | | | 0.31 | | 0.9 | remainder |
| 8005a | | | | | | | | | |
| 8006 | 63.8 | 2.8 | 2.9 | | | 0.06 | 0.07 | 2.1 | remainder |
| 8008a | | | | | | | | | |
| 8007 | 71.5 | 3.9 | 1.5 | | | | 0.20 | 1.4 | remainder |
| 8007a | | | | | | | | | |
| 8008 | 64.2 | 2.9 | 2.4 | 0.3 | 0.28 | | | 2.1 | remainder |
| 8008a | | | | | | | | | |
| 8009 | 68.8 | 3.4 | 1.0 | 1.5 | 0.07 | 0.20 | | 1.7 | remainder |
| 8009a | | | | | | | | | |
| 8010 | 65.3 | 3.6 | 2.8 | 0.2 | 0.05 | | 0.13 | 2.2 | remainder |
| 8010a | | | | | | | | | |

**Table 5**

| No. | alloy composition (wt%) | | | | | | | | | |
|---|---|---|---|---|---|---|---|---|---|---|
| | Cu | Si | Sn | Al | Bi | Te | Se | P | Mn | Zn |
| 8011 | 66.8 | 3.3 | 1.9 | 2.1 | 0.04 | 0.05 | 0.05 | | 2.3 | remainder |
| 8011a | | | | | | | | | | |
| 8012 | 75.1 | 4.1 | 0.4 | 2.4 | | 0.03 | | | 1.8 | remainder |
| 8012a | | | | | | | | | | |
| 8013 | 74.2 | 3.9 | 0.5 | 1.8 | | 0.10 | 0.04 | | 1.7 | remainder |
| 8013a | | | | | | | | | | |
| 8014 | 77.1 | 4.2 | 0.4 | 2.1 | | | 0.32 | | 2.0 | remainder |
| 8014a | | | | | | | | | | |
| 8015 | 62.8 | 2.6 | 2.9 | | 0.12 | | | 0.03 | 1.2 | remainder |
| 8015a | | | | | | | | | | |
| 8016 | 64.4 | 2.9 | 2.7 | | 0.23 | 0.09 | | 0.13 | 1.8 | remainder |
| 8016a | | | | | | | | | | |
| 8017 | 68.3 | 3.6 | 0.4 | | 0.05 | | 0.05 | 104 | 2.2 | remainder |
| 8017a | | | | | | | | | | |
| 8018 | 73. 2 | 4.3 | 0.5 | | 0.06 | 0.02 | 0.11 | 0.02 | 3.1 | remainder |
| 8018a | | | | | | | | | | |
| 8019 | 72.4 | 4.1 | 0.7 | | | 0.14 | | 0.21 | 2.1 | remainder |
| 8019a | | | | | | | | | | |
| 8020 | 69.5 | 3.7 | 0.7 | | | 0.06 | 0.04 | 0.05 | 1.9 | remainder |
| 8020a | | | | | | | | | | |

**Table 6**

| No. | alloy composition (wt%) | | | | | | | | | |
|---|---|---|---|---|---|---|---|---|---|---|
| | Cu | Si | Sn | Al | Bi | Te | Se | P | Mn | Zn |
| 8021 | 64.2 | 3.4 | 2.5 | | | | 0.31 | 0.03 | 1.9 | remainder |
| 8021a | | | | | | | | | | |
| 8022 | 65.6 | 3.7 | 2.3 | 0.2 | 0.06 | | | 0.03 | 1.4 | remainder |
| 8022a | | | | | | | | | | |
| 8023 | 67.1 | 3.6 | 0.4 | 0.5 | 0.04 | 0.05 | | 0.05 | 2.0 | remainder |
| 8023a | | | | | | | | | | |
| 8024 | 73.2 | 4.0 | 0.5 | 2.1 | 0.03 | | 0.05 | 0.12 | 2.4 | remainder |
| 8024a | | | | | | | | | | |
| 8025 | 68.8 | 3.5 | 0.4 | 1.8 | 0.12 | 0.03 | 0.03 | 0.04 | 1.8 | remainder |
| 8025a | | | | | | | | | | |
| 8026 | 66. 5 | 3.4 | 1.2 | 0.3 | | 0.24 | | 0.21 | 1.7 | remainder |
| 8026a | | | | | | | | | | |
| 8027 | 64.8 | 3.0 | 1.3 | 1.2 | | 0.16 | 0.10 | 0.06 | 1.5 | remainder |
| 8027a | | | | | | | | | | |
| 8028 | 71.2 | 3.9 | 0.4 | 1.0 | | | 0.14 | 0.03 | 2.6 | remainder |
| 8028a | | | | | | | | | | |
| 8029 | 68.1 | 3.6 | | 0.2 | 0.05 | | | | 2.0 | remainder |
| 8029a | | | | | | | | | | |
| 8030 | 64.9 | 2.9 | | 0.3 | 0.28 | 0. 08 | | | 1.0 | remainder |
| 8030a | | | | | | | | | | |

**Table 7**

| No. | alloy composition (wt%) | | | | | | | | |
|---|---|---|---|---|---|---|---|---|---|
| | Cu | Si | Al | Bi | Te | Se | P | Mn | Zn |
| 8031 | 75.3 | 3.9 | 2.1 | 0.07 | | 0.04 | | 0.8 | remainder |
| 8031a | | | | | | | | | |
| 8032 | 77.2 | 4.3 | 2.3 | 0.03 | 0.25 | 0.04 | | 2.8 | remainder |
| 8032a | | | | | | | | | |
| 8033 | 64.7 | 2. 8 | 2.2 | | 0.33 | | | 0. 9 | remainder |
| 8033a | | | | | | | | | |
| 8034 | 69.3 | 3.5 | 1.6 | | 0.03 | 0.03 | | 1.8 | remainder |
| 8034a | | | | | | | | | |
| 8035 | 71.2 | 3.8 | 1.5 | | | 0.21 | | 2.0 | remainder |
| 8035a | | | | | | | | | |
| 8036 | 70.6 | 3.7 | 0.3 | 0.04 | | | 0.13 | 1.7 | remainder |
| 8036a | | | | | | | | | |
| 8037 | 69.7 | 3.8 | 1.4 | 0.12 | 0.04 | | 0.04 | 1.8 | remainder |
| 8037a | | | | | | | | | |
| 8038 | 70.7 | 4.2 | 1.5 | 0.03 | | 0.16 | 0.03 | 3.3 | remainder |
| 8038a | | | | | | | | | |
| 8039 | 70.4 | 3.9 | 0.2 | 0.15 | 0.10 | 0.02 | 0.04 | 2.2 | remainder |
| 8039a | | | | | | | | | |
| 8040 | 68.8 | 3.7 | 0.4 | | 0.05 | | 0.12 | 1.9 | remainder |
| 8040a | | | | | | | | | |

**Table 8**

| No. | alloy composition (wt%) | | | | | | | | | | |
|---|---|---|---|---|---|---|---|---|---|---|---|
| | Cu | Si | Sn | Al | Bi | Te | Se | P | Mn | Ni | Zn |
| 8041 | 70.3 | 3.9 | | 0.2 | | 0.20 | 0.03 | 0.22 | 2.1 | | remainder |
| 8041a | | | | | | | | | | | |
| 8042 | 74.6 | 4.3 | | 2.1 | | | 0.12 | 0.03 | 2.4 | | remainder |
| 8042a | | | | | | | | | | | |
| 8043 | 77.0 | 4. 5 | | | 0.03 | | | 0.12 | 1.7 | | remainder |
| 8043a | | | | | | | | | | | |
| 8044 | 70.6 | 3.9 | | | 0.10 | 0.06 | | 0.04 | 2.6 | | remainder |
| 8044a | | | | | | | | | | | |
| 8045 | 74.2 | 4.3 | | | 0.11 | | 0.21 | 0.16 | 2.8 | | remainder |
| 8045a | | | | | | | | | | | |
| 8046 | 69.9 | 3.8 | | | 0.06 | 0.11 | 0.03 | 0.08 | 1.2 | | remainder |
| 8046a | | | | | | | | | | | |
| 8047 | 66.8 | 3.4 | | | | 0.09 | | 0.06 | 2.2 | | remainder |
| 8047a | | | | | | | | | | | |
| 8048 | 71.3 | 4. 2 | | | | 0.04 | 0.05 | 0.05 | 1.4 | | remainder |
| 8048a | | | | | | | | | | | |
| 8049 | 72.4 | 4.1 | | | | | 0.12 | 0.09 | 2.7 | | remainder |
| 8049a | | | | | | | | | | | |
| 8050 | 62.9 | 2.8 | 2.8 | | 0.12 | | | | | 1.5 | remainder |
| 8050a | | | | | | | | | | | |

**Table 9**

| No. | alloy composition (wt%) | | | | | | | | |
|---|---|---|---|---|---|---|---|---|---|
| | Cu | Si | Sn | Al | Bi | Te | Se | Ni Zn | |
| 8051 | 64.8 | 3.1 | 2.4 | | 0.08 | 0.03 | | 2.0 | remainder |
| 8051a | | | | | | | | | |
| 8052 | 68.9 | 3.9 | 0.3 | | 0.03 | | 0.06 | 1.8 | remainder |
| 8052a | | | | | | | | | |
| 8053 | 67.3 | 3.7 | 0.7 | | 0.05 | 0.04 | 0.04 | 2.1 | remainder |
| 8053a | | | | | | | | | |
| 8054 | 66.5 | 3.8 | 0.9 | | | 0.31 | | 2.2 | remainder |
| 8054a | | | | | | | | | |
| 8055 | 73.8 | 4.3 | 2.1 | | | 0.03 | 0.05 | 3.3 | remainder |
| 8055a | | | | | | | | | |
| 8056 | 74.2 | 4.4 | 1.3 | | | | 0.03 | 2.7 | remainder |
| 8056a | | | | | | | | | |
| 8057 | 70.1 | 3.8 | 1.5 | 1.9 | 0.06 | | | 1.8 | remainder |
| 8057a | | | | | | | | | |
| 8058 | 67.9 | 2.9 | 0.8 8 | 2.3 | 0.16 | 0.06 | | 0.9 | remainder |
| 8058a | | | | | | | | | |
| 8059 | 68.2 | 3.6 | 2.0 | 0.6 | 0.04 | | 0.09 | 1.7 | remainder |
| 8059a | | | | | | | | | |
| 8060 | 66.6 | 3.5 | 1.8 | 0.2 | 0.10 | 0.05 | 0.05 | 1.2 | remainder |
| 8060a | | | | | | | | | |

**Table 10**

| No. | alloy composition (wt%) | | | | | | | | | |
|---|---|---|---|---|---|---|---|---|---|---|
| | Cu | Si | Sn | Al | Bi | Te | Se | P | Ni | Zn |
| 8061 | 67.6 | 3.6 | 0.44 | 0.6 | | 0.30 | | | 1.8 | remainder |
| 8061a | | | | | | | | | | |
| 8062 | 68. 8 | 3.0 | 0.6 | 2.1 | | 0.08 | 0.03 | | 1.1 | remainder |
| 8062a | | | | | | | | | | |
| 8063 | 71.2 | 4.1 | 2.4 | 0.8 | | | 0.31 | | 2.2 | remainder |
| 8063a | | | | | | | | | | |
| 8064 | 68.2 | 3.6 | 2.6 | | 0.04 | | | 0.05 | 1.5 | reminder |
| 8064a | | | | | | | | | | |
| 8065 | 63.9 | 2.9 | 2.3 | | 0.32 | 0.02 | | 0.08 | 0.8 | reminder |
| 8065a | | | | | | | | | | |
| 8066 | 70.5 | 3.9 | 1.1 | | 0.05 | | 0.05 | 0.05 | 2.2 | remainder |
| 8066a | | | | | | | | | | |
| 8067 | 67.7 | 3.7 | 12 | | 0.09 | 0.03 | 0.02 | 0.04 | 2.0 | remainder |
| 8067a | | | | | | | | | | |
| 8068 | 66.6 | 3.5 | 1.4 | | | 0.06 | | 0.04 | 2.6 | remainder |
| 8068a | | | | | | | | | | |
| 8069 | 72.3 | 4.1 | 0.6 | | | 0.05 | 0.04 | 0.10 | 3.0 | remainder |
| 8069a | | | | | | | | | | |
| 8070 | 70.6 | 4.0 | 0.4 | | | | 0.16 | 0.05 | 3.2 | remainder |
| 8070a | | | | | | | | | | |

**Table 11**

| No. | alloy opposition (wt%) | | | | | | | | | |
|---|---|---|---|---|---|---|---|---|---|---|
| | Cu | Si | Sn | Al | Bi | Te | Se | P | Ni | Zn |
| 8071 | 75.6 | 3.9 | 0.5 | 2.2 | 0.21 | | | 0.21 | 1.4 | remainder |
| 8071a | | | | | | | | | | |
| 8072 | 71.2 | 3.4 | 0.7 | 1.5 | 0.18 | 0.10 | | 0.14 | 1.3 | remainder |
| 8072a | | | | | | | | | | |
| 8073 | 68.5 | 3.7 | 0.7 | 1.2 | 0.03 | | 0.08 | 0.03 | 1.9 | remainder |
| 8073a | | | | | | | | | | |
| 8074 | 64.9 | 3.2 | 0.8 | 0.4 | 0.12 | 0.03 | 0.04 | 0.04 | 1.8 | remainder |
| 8074a | | | | | | | | | | |
| 8075 | 65.3 | 3.3 | 2.8 | 0.2 | | 0.06 | | 0.05 | 1.5 | remainder |
| 8075a | | | | | | | | | | |
| 8076 | 68.8 | 4.0 | 2.5 | 0.6 | | 0.05 | 0.13 | 0.03 | 2.7 | remainder |
| 8076a | | | | | | | | | | |
| 8077 | 67.3 | 3.4 | 1.6 | 0.5 | | | 0.06 | 0.12 | 2.4 | remainder |
| 8077a | | | | | | | | | | |
| 8078 | 77.0 | 4.1 | | 2.2 | 0.13 | | | | 2.1 | remainder |
| 8078a | | | | | | | | | | |
| 8079a | 71.2 | 3.8 | | 1.4 | 0.05 | 0.20 | | | 2.0 | remainder |
| 8079a | | | | | | | | | | |
| 8080 | 68.2 | 3.8 | | 1.3 | 0.04 | | 0.05 | | 2.8 | remainder |
| 8080a | | | | | | | | | | |

**Table 12**

| No. | alloy composition(wt%) | | | | | | | | |
|---|---|---|---|---|---|---|---|---|---|
| | Cu | Si | Al | Bi | Te | Se | P | Ni | Zn |
| 8081 | 67.3 | 3.4 | 0.8 | 0.05 | 0.06 | 0.03 | | 1.7 | remainder |
| 8081a | | | | | | | | | |
| 8082 | 70.4 | 3.9 | 1.2 | | 0.05 | | | 2.2 | remainder |
| 8082a | | | | | | | | | |
| 8083 | 73.6 | 3.9 | 1.3 | | 0.21 | 0.06 | | 3.1 | remainder |
| 8083a | | | | | | | | | |
| 8084 | 68.8 | 3.8 | 1.2 | | | 0.18 | | 2.6 | remainder |
| 8084a | | | | | | | | | |
| 8085 | 67.5 | 3.5 | 1.2 | 0.04 | | | 0.16 | 1.8 | remainder |
| 8085a | | | | | | | | | |
| 8086 | 64.9 | 2.9 | 1.6 | 0.08 | 0.04 | | 0.05 | 1.5 | remainder |
| 8086a | | | | | | | | | |
| 8087 | 76.3 | 4.3 | 1.5 | 0.29 | | 0.05 | 0.10 | 2.8 | remainder |
| 8087a | | | | | | | | | |
| 8088 | 65.8 | 2.8 | 2.3 | 0.16 | 0.06 | 0.03 | 0.05 | 1.3 | remainder |
| 8088a | | | | | | | | | |
| 8089 | 66.7 7 | 3.3 | 2.1 | | 0.32 | | 0.03 | 1.8 | remainder |
| 8089a | | | | | | | | | |
| 8090 | 69.2 | 4.0 | 1.2 | | 0.11 | 0.02 | 0.10 | 2.5 | remainder |
| 8090a | | | | | | | | | |

**Table 13**

| No. | alloy composition (wt%) | | | | | | | | | | |
|---|---|---|---|---|---|---|---|---|---|---|---|
| | Cu | Si | Sn | Al | Bi | Te | Se | P | Mn | Ni | Zn |
| 8091 | 70.6 | 3.8 | | 1.3 | | | 0.14 | 0.05 | | 1.7 | remainder |
| 8091a | | | | | | | | | | | |
| 8092 | 67.2 | 3.4 | | | 0.05 | | | 0.04 | | 2. 0 | remainder |
| 8092a | | | | | | | | | | | |
| 8093 | 65.8 | 3.2 | | | 0.15 | 0.03 | | 0.06 | | 1.2 | remainder |
| 8093a | | | | | | | | | | | |
| 8094 | 67.7 | 3.7 | | | 0.06 | | 0.10 | 0.08 | | 2.1 | remainder |
| 8094a | | | | | | | | | | | |
| 8095 | 64.7 | 2.9 | | | 0.31 | 0.04 | 0.05 | 0.09 | | 1.5 | remainder |
| 8095a | | | | | | | | | | | |
| 8096 | 66.5 | 3.6 | | | | 0.18 | | 0.21 | | 2.3 | remainder |
| 8096a | | | | | | | | | | | |
| 8097 | 67.3 | 3.8 | | | | 0.08 | 0.05 | 0.12 | | 2.2 | remainder |
| 8097a | | | | | | | | | | | |
| 8098 | 65.9 | 3.6 | | | | | 0.21 | 0.20 | | 2.5 | remainder |
| 8098a | | | | | | | | | | | |
| 8099 | 64.9 | 3.6 | 0.4 | | 0.18 | | | | 0.8 | 2.6 | remainder |
| 8099a | | | | | | | | | | | |
| 8100 | 67.3 | 3.8 | 1.8 | | 0.03 | 0.06 | | | 1.9 | 1.0 | remainder |
| 8100a | | | | | | | | | | | |

**Table 14**

| No. | alloy composition (wt%) | | | | | | | | | |
|---|---|---|---|---|---|---|---|---|---|---|
| | Cu | Si | Sn | Al | Bi | Te | Se | Mn | Ni | Zn |
| 8101 | 62.9 | 2.9 | 2.4 | | 0.20 | | 0.16 | 1.3 | 0.9 | remainder |
| 8101a | | | | | | | | | | |
| 8102 | 68.3 | 3.4 | 0.5 | | 0.04 | 0.04 | 0.05 | 1.5 | 0.8 | remainder |
| 8102a | | | | | | | | | | |
| 8103 | 65.8 | 3.8 | 2.6 | | | 0.03 | | 1.4 | 1.2 | remainder |
| 8103a | | | | | | | | | | |
| 8104 | 64.7 | 3.6 | 2.7 | | | 0.25 | 0.03 | 1.3 | 1.6 | remainder |
| 8104a | | | | | | | | | | |
| 8105 | 70.4 | 3.9 | 1.8 | | | | 0.07 | 1.0 | 2.0 | remainder |
| 8105a | | | | | | | | | | |
| 8106 | 70.3 | 3.8 | 0.4 | 1.8 | 0.05 | | | 2.3 | 0.7 | remainder |
| 8106a | | | | | | | | | | |
| 8107 | 72.1 | 3.7 | 0.4 | 2.1 | 0.03 | 0.05 | | 1.3 | 1.2 | remainder |
| 8107a | | | | | | | | | | |
| 8108 | 69.8 | 3.8 | 0.6 | 1.5 | 0.05 | | 0.05 | 1.5 | 2.1 | remainder |
| 8108a | | | | | | | | | | |
| 8109 | 75.4 | 4.2 | 0.6 | 1.8 | 0.05 | 0.04 | 0.04 | 2.3 | 1.1 | remainder |
| 8109a | | | | | | | | | | |
| 8110 | 66.4 | 3.5 | 2.5 | 0.2 | | 0.12 | | 1.6 | 0.9 | remainder |
| 8110a | | | | | | | | | | |

**Table 15**

| No. | alloy composition (wt%) | | | | | | | | | | |
|---|---|---|---|---|---|---|---|---|---|---|---|
| | Cu | Si | Sn | Al | Bi | Te | Se | P | Mn | Ni | Zn |
| 8111 | 64.9 | 3.3 | 2.5 | 0.3 | | 0.08 | 0.05 | | 1.2 | 1.3 | remainder |
| 8111a | | | | | | | | | | | |
| 8112 | 70.0 | 3.8 | 1.2 | 0.5 | | | 0.03 | | 1.5 | 0.8 | remainder |
| 8112a | | | | | | | | | | | |
| 8113 | 72.0 | 3.9 | 1.1 | | 0.25 | | | 0.20 | 2.4 | 0.9 | remainder |
| 8113a | | | | | | | | | | | |
| 8114 | 66.5 | 3.6 | 1.2 | | 0.06 | 0.04 | | 0.05 | 1.3 | 1.1 | remainder |
| 8114a | | | | | | | | | | | |
| 8115 | 67.0 | 3.5 | 1.3 | | 0.12 | | 0.04 | 0.08 | 0.9 | 1.2 | remainder |
| 8115a | | | | | | | | | | | |
| 8116 | 64.0 | 2.8 | 2.6 | | 0.30 | 0.08 | 0.03 | 0.05 | 0.8 | 1.0 | remainder |
| 8116a | | | | | | | | | | | |
| 8117 | 67.3 | 3.7 | 2.3 | | | 0.03 | | 0.03 | 1.2 | 1.3 | remainder |
| 8117a | | | | | | | | | | | |
| 8118 | 66.4 | 3.8 | 2.4 | | | 0.05 | 0.15 | 0.03 | 1.0 | 1.6 | remainder |
| 8118a | | | | | | | | | | | |
| 8119 | 70.2 | 3.9 | 0.5 | | | | 0.30 | 0.07 | 1.7 | 0.9 | remainder |
| 8119a | | | | | | | | | | | |
| 8120 | 73.1 | 4.2 | 0.5 | 2.3 | 0.04 | | | 4.14 | 2.00 | 1.1 | remainder |
| 8120a | | | | | | | | | | | |

**Table 16**

| No. | alloy composition (wt%) | | | | | | | | | | |
|---|---|---|---|---|---|---|---|---|---|---|---|
| | Cu | Si | Sn | Al | Bi | Te | Se | P | Mn | Ni | Zn |
| 8121 | 71.0 | 3.6 | 0.6 | 2.3 | 0.03 | 0.12 | | 0.20 | 1.8 | 1.3 | remainder |
| 8121a | | | | | | | | | | | |
| 8122 | 70.0 | 3.5 | 0.5 | 1.8 | 0.06 | | 0.03 | 0.10 | 1.2 | 1.3 | remainder |
| 8122a | | | | | | | | | | | |
| 8123 | 68.5 | 3.4 | 0.5 | 0.7 | 0.30 | 0.03 | 0.02 | 0.03 | 1.0 | 1.5 | remainder |
| 8123a | | | | | | | | | | | |
| 8124 | 68.8 | 3.9 | 1.2 | 0.2 | | 0.06 | | 0.05 | 1.0 | 1.2 | remainder |
| 8124a | | | | | | | | | | | |
| 8125 | 64.9 | 3.0 | 1.8 | 0.5 | | 0.25 | 0.05 | 0.05 | 1.1 | 0.8 | remainder |
| 8125a | | | | | | | | | | | |
| 8126 | 63.7 | 2.9 | 2.7 | 1.0 | | | 0.31 | 0.03 | 1.2 | 0.8 | remainder |
| 8126a | | | | | | | | | | | |
| 8127 | 70.4 | 3.9 | | 0.2 | 0.04 | | | | 1.6 | 1.3 | remainder |
| 8127a | | | | | | | | | | | |
| 8128 | 66.5 | 3.6 | | 0.3 | 0.02 | 0.04 | | | 1.2 | 1.1 | remainder |
| 8128a | | | | | | | | | | | |
| 8129 | 67.3 | 3.7 | | 0.7 | 0.03 | | 0.08 | | 1.3 | 1.2 | remainder |
| 8129a | | | | | | | | | | | |
| 8130 | 66.0 | 3.4 | | 0.7 | 0.22 | 0.08 | 0.04 | | 1.3 | 1.0 | remainder |
| 8130a | | | | | | | | | | | |

**Table 17**

| No. | alloy composition (wt%) | | | | | | | | | |
|---|---|---|---|---|---|---|---|---|---|---|
| | Cu | Si | Al | Bi | Te | Se | P | Mn | Ni | Zn |
| 8131 | 68.0 | 3.8 | 0.8 | | 0.05 | | | 1.1 | 1.4 | remainder |
| 8131a | | | | | | | | | | |
| 8132 | 70.0 | 3.4 | 2.1 | | 0.03 | 0.22 | | 0.9 | 1.1 | remainder |
| 8132a | | | | | | | | | | |
| 8133 | 75.5 | 4.2 | 2.2 | | | 0.05 | | 1.2 | 1.9 | remainder |
| 8133a | | | | | | | | | | |
| 8134 | 68.5 | 3.8 | 1.8 | 0.10 | | | 0.04 | 1.4 | 1.6 | remainder |
| 8134a | | | | | | | | | | |
| 8135 | 78.5 | 4.3 | 2.1 | 0.03 | 0.10 | | 0.15 | 1.8 | 1.3 | remainder |
| 8135a | | | | | | | | | | |
| 8136 | 66.5 | 3.6 | 1.2 | 0.05 | | 0.16 | 0.05 | 1.2 | 1.3 | remainder |
| 8136a | | | | | | | | | | |
| 8137 | 72.0 | 4.1 | 1.0 | 0.04 | 0.03 | 0.02 | 0.07 | 1.3 | 2.2 | remainder |
| 8137a | | | | | | | | | | |
| 8138 | 70.2 | 4.0 | 1.0 | | 0.04 | | 0.03 | 2.1 | 1.4 | remainder |
| 8138a | | | | | | | | | | |
| 8139 | 66.8 | 3.8 | 0.5 | | 0.32 | 0.03 | 0.03 | 1.2 | 1.6 | remainder |
| 8139a | | | | | | | | | | |
| 8140 | 67.3 | 3.9 | 0.4 | | | 0.05 | 0.03 | 1.8 | 1.0 | remainder |
| 8140a | | | | | | | | | | |

**Table 18**

| No. | alloy composition (wt%) | | | | | | | | |
|---|---|---|---|---|---|---|---|---|---|
| | Cu | Si | Bi | Te | Se | P | Mn | Ni | Zn |
| 8141 | 66.5 | 3.6 | 0.05 | | | 0.05 | 1.5 | 1.2 | remainder |
| 8141a | | | | | | | | | |
| 8142 | 63.9 | 2.9 | 0.30 | 0.03 | | 0.04 | 1.2 | 0.9 | remainder |
| 8142a | | | | | | | | | |
| 8143 | 68.4 | 3.8 | 0.03 | | 0.05 | 0.12 | 0.9 | 2.5 | remainder |
| 8143a | | | | | | | | | |
| 8144 | 65.8 | 3.4 | 0.10 | 0.05 | 0.02 | 0.03 | 1.0 | 1.4 | remainder |
| 8144a | | | | | | | | | |
| 8145 | 70.5 | 3.9 | | 0.12 | | 0.05 | 2.6 | 0.8 | remainder |
| 8145a | | | | | | | | | |
| 8146 | 72.0 | 4.2 | | 0.04 | 0.05 | 0.18 | 1.0 | 2.4 | remainder |
| 8146a | | | | | | | | | |
| 8147 | 68.0 | 3.7 | | | 0.20 | 0.06 | 1.5 | 1.0 | remainder |
| 8147a | | | | | | | | | |

**Table 19**

| No. | alloy composition (wt%) | | | | | | | | |
|---|---|---|---|---|---|---|---|---|---|
| | Cu | Si | Sn | Al | Mn | Pb | Fe | Ni | Zn |
| 14001 | 58.8 | | 0.2 | | | 3.1 | 0.2 | | remainder |
| 14001a | | | | | | | | | |
| 14002 | 61.4 | | 0.2 | | | 3.0 | 0.2 | | remainder |
| 14002a | | | | | | | | | |
| 14003 | 59.1 | | 0.2 | | | 2.0 | 0.2 | | remainder |
| 14003a | | | | | | | | | |
| 14004 | 69.2 | 1.2 | | | | 0.1 | | | remainder |
| 14004a | | | | | | | | | |
| 14005 | remainder | | | 9.8 | 1.1 | | 3.9 | 1.2 | |
| 14005a | | | | | | | | | |
| 14006 | 61.8 | | 1.0 | | | 0.1 | | | remainder |
| 14006a | | | | | | | | | |

**Table 20**

| No. | machinability | | | hot workability | mechanical properties | |
|---|---|---|---|---|---|---|
| | form of chippings | condition of cut surface | cutting force (N) | 700°C deformability | tensile strength (N/mm²) | elongation (%) |
| 7001 | ⊚ | Δ | 138 | ○ | 670 | 18 |
| 7002 | ⊚ | Δ | 136 | ○ | 712 | 20 |
| 7003 | ⊚ | ○ | 132 | ○ | 783 | 23 |
| 7004 | ⊚ | ○ | 138 | ○ | 736 | 21 |
| 7005 | ⊚ | ○ | 136 | ○ | 785 | 23 |
| 7006 | ⊚ | Δ | 139 | ○ | 700 | 24 |
| 7007 | Δ | ○ | 138 | ○ | 707 | 23 |
| 7008 | ⊚ | ○ | 131 | ○ | 805 | 22 |
| 7009 | ⊚ | ○ | 136 | ○ | 768 | 19 |
| 7010 | ⊚ | ○ | 135 | ○ | 718 | 23 |
| 7011 | Δ | ○ | 137 | ○ | 677 | 23 |
| 7012 | ⊚ | ○ | 134 | ○ | 800 | 21 |
| 7013 | ⊚ | ○ | 133 | ○ | 819 | 22 |
| 7014 | Δ | ○ | 138 | ○ | 641 | 21 |
| 7015 | ⊚ | ○ | 134 | ○ | 764 | 23 |
| 7010 | ⊚ | ○ | 129 | ○ | 759 | 20 |
| 7017 | Δ | ○ | 139 | ○ | 638 | 18 |
| 7018 | ⊚ | ○ | 135 | ○ | 717 | 20 |
| 7019 | ⊚ | ○ | 136 | ○ | 694 | 24 |
| 7020 | Δ | ○ | 138 | ○ | 712 | 25 |

**Table 21**

| No. | machinability | | | hot workability | mechanical properties | |
|---|---|---|---|---|---|---|
| | form of chippings | condition of cut surface | cutting force (N) | 700°C deformability | tensile strength (N/mm²) | elongation (%) |
| 7021 | ⊚ | ○ | 130 | ○ | 754 | 24 |
| 7022 | ⊚ | Δ | 134 | ○ | 780 | 23 |
| 7023 | ⊚ | ○ | 133 | ○ | 765 | 22 |
| 7024 | ⊚ | ○ | 135 | ○ | 772 | 23 |
| 7025 | Δ | ○ | 138 | ○ | 687 | 24 |
| 7026 | ⊚ | ○ | 135 | ○ | 718 | 24 |
| 7027 | ⊚ | Δ | 136 | ○ | 742 | 18 |
| 7028 | Δ | ○ | 138 | ○ | 785 | 20 |
| 7029 | ⊚ | ○ | 134 | ○ | 703 | 23 |
| 7030 | ⊚ | ○ | 135 | ○ | 820 | 18 |

**Table 22**

| No. | machinability | | | hot workability | mechanical properties | |
|---|---|---|---|---|---|---|
| | form of chippings | condition of cut surface | cutting force (N) | 700 °C deformability | tensile strength (N/mm²) | elongation (%) |
| 8001 | ⊚ | ○ | 132 | ○ | 655 | 15 |
| 8002 | ⊚ | ○ | 129 | ○ | 708 | 17 |
| 8003 | ⊚ | ○ | 127 | ○ | 768 | 20 |
| 8004 | ⊚ | ○ | 128 | ○ | 785 | 18 |
| 8005 | ⊚ | ○ | 131 | ○ | 714 | 16 |
| 8006 | ⊚ | ○ | 134 | ○ | 680 | 16 |
| 8007 | ⊚ | ○ | 132 | ○ | 764 | 17 |
| 8008 | ⊚ | ○ | 130 | ○ | 673 | 16 |
| 8009 | ⊚ | ○ | 132 | ○ | 759 | 18 |
| 8010 | ⊚ | ○ | 132 | ○ | 751 | 15 |
| 8011 | ⊚ | ○ | 134 | ○ | 767 | 17 |
| 8012 | ⊚ | ○ | 128 | ○ | 796 | 18 |
| 8013 | ⊚ | ○ | 129 | ○ | 784 | 18 |
| 8014 | ⊚ | ○ | 129 | ○ | 802 | 17 |
| 8015 | ⊚ | ○ | 133 | ○ | 679 | 15 |
| 8016 | ⊚ | ○ | 130 | ○ | 706 | 16 |
| 8017 | ⊚ | ○ | 129 | ○ | 707 | 18 |
| 8018 | ⊚ | ○ | 131 | ○ | 780 | 16 |
| 8019 | ⊚ | ○ | 128 | ○ | 768 | 16 |
| 8020 | ⊚ | ○ | 132 | ○ | 723 | 19 |

**Table 23**

| No. | machinability | | | hot workability | mechanical properties | |
|---|---|---|---|---|---|---|
| | form of chippings | condition of cut surface | cutting force (N) | 700°C deformability | tensile strength (N/mm²) | elongation (%) |
| 8021 | ⊚ | ○ | 134 | ○ | 765 | 16 |
| 8022 | ⊚ | ○ | 132 | ○ | 770 | 16 |
| 8023 | ⊚ | ○ | 131 | ○ | 746 | 18 |
| 8024 | ⊚ | ○ | 132 | ○ | 816 | 19 |
| 8025 | ⊚ | ○ | 129 | ○ | 159 | 18 |
| 8026 | ⊚ | ○ | 130 | ○ | 726 | 17 |
| 8027 | ⊚ | ○ | 133 | ○ | 703 | 17 |
| 8028 | ⊚ | ○ | 132 | ○ | 737 | 18 |
| 8029 | ⊚ | ○ | 129 | ○ | 719 | 20 |
| 8030 | ⊚ | ○ | 133 | ○ | 645 | 23 |
| 8031 | ⊚ | ○ | 129 | ○ | 764 | 22 |
| 8032 | ⊚ | ○ | 131 | ○ | 790 | 19 |
| 8033 | ⊚ | ○ | 133 | ○ | 674 | 20 |
| 8034 | ⊚ | ○ | 131 | ○ | 748 | 23 |
| 8035 | ⊚ | ○ | 129 | ○ | 777 | 22 |
| 8036 | ⊚ | ○ | 131 | ○ | 725 | 23 |
| 8037 | ⊚ | ○ | 128 | ○ | 770 | 21 |
| 8038 | ⊚ | ○ | 131 | ○ | 815 | 18 |
| 8039 | ⊚ | ○ | 127 | ○ | 739 | 24 |
| 8040 | ⊚ | ○ | 130 | ○ | 721 | 22 |

**Table 24**

| No. | machinability | | | hot workability | mechanical properties | |
|---|---|---|---|---|---|---|
| | form of chippings | condition of cut surface | cutting force (N) | 700°C deformability | tensile strength (N/mm²) | elongation (%) |
| 8041 | ⊚ | ○ | 128 | ○ | 735 | 23 |
| 8042 | ⊚ | ○ | 127 | ○ | 822 | 18 |
| 8043 | ⊚ | ○ | 131 | ○ | 780 | 18 |
| 8044 | ⊚ | ○ | 126 | ○ | 726 | 21 |
| 8045 | ⊚ | ○ | 128 | ○ | 766 | 22 |
| 8046 | ⊚ | ○ | 127 | ○ | 712 | 23 |
| 8047 | ⊚ | ○ | 128 | ○ | 674 | 21 |
| 8048 | ⊚ | ○ | 129 | ○ | 753 | 24 |
| 8049 | ⊚ | ○ | 127 | ○ | 768 | 22 |
| 8050 | ⊚ | ○ | 132 | ○ | 691 | 17 |
| 8051 | ⊚ | ○ | 131 | ○ | 717 | 17 |
| 8052 | ⊚ | ○ | 128 | ○ | 739 | 21 |
| 8053 | ⊚ | ○ | 128 | ○ | 730 | 22 |
| 8054 | ⊚ | ○ | 127 | ○ | 735 | 20 |
| 8055 | ⊚ | ○ | 134 | ○ | 818 | 15 |
| 8056 | ⊚ | ○ | 132 | ○ | 812 | 16 |
| 8057 | ⊚ | ○ | 131 | ○ | 755 | 18 |
| 8058 | ⊚ | ○ | 133 | ○ | 659 | 20 |
| 8059 | ⊚ | ○ | 132 | ○ | 740 | 17 |
| 8060 | ⊚ | ○ | 130 | ○ | 714 | 19 |

**Table 25**

| No. | machinability | | | hot workability | mechanical properties | |
|---|---|---|---|---|---|---|
| | form of chippings | condition of cut surface | cutting force (N) | 700°C deformability | tensile strength (N/mm²) | elongation (%) |
| 8061 | ⊚ | ○ | 129 | ○ | 705 | 21 |
| 8062 | ⊚ | ○ | 131 | ○ | 690 | 22 |
| 8063 | ⊚ | ○ | 133 | ○ | 811 | 18 |
| 8064 | ⊚ | ○ | 131 | ○ | 746 | 17 |
| 8065 | ⊚ | ○ | 133 | ○ | 652 | 19 |
| 8066 | ⊚ | ○ | 130 | ○ | 758 | 19 |
| 8067 | ⊚ | ○ | 129 | ○ | 734 | 19 |
| 8068 | ⊚ | ○ | 131 | ○ | 710 | 17 |
| 8069 | ⊚ | ○ | 131 | ○ | 767 | 20 |
| 8070 | ⊚ | ○ | 131 | ○ | 753 | 18 |
| 8071 | ⊚ | ○ | 129 | ○ | 792 | 19 |
| 8072 | ⊚ | ○ | 131 | ○ | 736 | 21 |
| 8073 | ⊚ | ○ | 130 | ○ | 767 | 22 |
| 8074 | ⊚ | ○ | 132 | ○ | 679 | 19 |
| 8075 | ⊚ | ○ | 134 | ○ | 728 | 17 |
| 8076 | ⊚ | ○ | 133 | ○ | 795 | 16 |
| 8077 | ⊚ | ○ | 133 | ○ | 716 | 18 |
| 8078 | ⊚ | ○ | 132 | ○ | 809 | 18 |
| 8079 | ⊚ | ○ | 129 | ○ | 758 | 22 |
| 8080 | ⊚ | ○ | 130 | ○ | 724 | 21 |

**Table 26**

| No. | machinability | | | hot workability | mechanical properties | |
|---|---|---|---|---|---|---|
| | form of chippings | condition of cut surface | cutting force (N) | 700°C deformability | tensile strength (N/mm²) | elongation (%) |
| 8081 | ⊚ | ○ | 132 | ○ | 706 | 23 |
| 8082 | ⊚ | ○ | 130 | ○ | 768 | 23 |
| 8083 | ⊚ | ○ | 128 | ○ | 774 | 25 |
| 8084 | ⊚ | ○ | 129 | ○ | 765 | 22 |
| 8085 | ⊚ | ○ | 130 | ○ | 729 | 23 |
| 8086 | ⊚ | ○ | 133 | ○ | 687 | 24 |
| 8087 | ⊚ | ○ | 131 | ○ | 798 | 20 |
| 8088 | ⊚ | ○ | 132 | O | 699 | 23 |
| 8089 | ⊚ | ○ | 130 | ○ | 740 | 21 |
| 8090 | ⊚ | ○ | 132 | ○ | 782 | 18 |
| 8091 | ⊚ | ○ | 129 | ○ | 763 | 22 |
| 8092 | ⊚ | ○ | 130 | ○ | 680 | 22 |
| 8093 | ⊚ | ○ | 131 | ○ | 655 | 23 |
| 8094 | ⊚ | ○ | 128 | ○ | 714 | 21 |
| 8095 | ⊚ | ○ | 132 | ○ | 638 | 24 |
| 8096 | ⊚ | ○ | 128 | ○ | 889 | 22 |
| 8097 | ⊚ | ○ | 129 | ○ | 711 | 21 |
| 8098 | ⊚ | ○ | 130 | ○ | 893 | 20 |
| 8099 | ⊚ | ○ | 127 | ○ | 702 | 21 |
| 8100 | ⊚ | ○ | 129 | ○ | 724 | 18 |

**Table 27**

| No. | machinability | | | hot workability | mechanical properties | |
|---|---|---|---|---|---|---|
| | form of chippings | condition of cut surface | cutting force (N) | 700°C deformability | tensile strength (N/mm²) | elongation (%) |
| 8101 | ⊚ | ○ | 131 | ○ | 685 | 18 |
| 8102 | ⊚ | ○ | 132 | ○ | 690 | 21 |
| 8103 | ⊚ | ○ | 133 | ○ | 744 | 17 |
| 8104 | ⊚ | ○ | 130 | ○ | 726 | 17 |
| 8105 | ⊚ | ○ | 133 | ○ | 751 | 19 |
| 8106 | ⊚ | ○ | 130 | ○ | 752 | 21 |
| 8107 | ⊚ | ○ | 131 | ○ | 760 | 21 |
| 8108 | ⊚ | ○ | 132 | ○ | 748 | 22 |
| 8109 | ⊚ | ○ | 130 | ○ | 807 | 18 |
| 8110 | ⊚ | ○ | 133 | ○ | 739 | 16 |
| 8111 | ⊚ | ○ | 132 | ○ | 717 | 17 |
| 8112 | ⊚ | ○ | 134 | ○ | 763 | 20 |
| 8113 | ⊚ | ○ | 129 | ○ | 745 | 22 |
| 8114 | ⊚ | ○ | 132 | ○ | 722 | 20 |
| 8115 | ⊚ | ○ | 130 | ○ | 706 | 17 |
| 8116 | ⊚ | ○ | 133 | ○ | 684 | 19 |
| 8117 | ⊚ | ○ | 132 | ○ | 740 | 18 |
| 8118 | ⊚ | ○ | 133 | ○ | 765 | 16 |
| 8119 | ⊚ | ○ | 128 | ○ | 733 | 22 |
| 8120 | ⊚ | ○ | 131 | ○ | 819 | 19 |

**Table 28**

| No. | machinability | | | hot workability | mechanical properties | |
|---|---|---|---|---|---|---|
| | form of chippings | condition of cut surface | cutting force (N) | 700°C deformability | tensile strength (N/mm²) | elongation (%) |
| 8121 | ⊚ | ○ | 130 | ○ | 788 | 20 |
| 8122 | ⊚ | ○ | 131 | ○ | 755 | 22 |
| 8123 | ⊚ | ○ | 127 | ○ | 711 | 21 |
| 8124 | ⊚ | ○ | 130 | ○ | 763 | 20 |
| 8125 | ⊚ | ○ | 131 | ○ | 687 | 18 |
| 8126 | ⊚ | ○ | 134 | ○ | 706 | 17 |
| 8127 | ⊚ | ○ | 128 | ○ | 730 | 22 |
| 8128 | ⊚ | ○ | 130 | ○ | 702 | 23 |
| 8129 | ⊚ | ○ | 132 | ○ | 727 | 21 |
| 8130 | ⊚ | ○ | 130 | ○ | 701 | 24 |
| 8131 | ⊚ | ○ | 129 | ○ | 745 | 22 |
| 8132 | ⊚ | ○ | 132 | ○ | 749 | 21 |
| 8133 | ⊚ | ○ | 130 | ○ | 826 | 18 |
| 8134 | ⊚ | ○ | 128 | ○ | 770 | 20 |
| 8135 | ⊚ | ○ | 129 | ○ | 828 | 17 |
| 8136 | ⊚ | ○ | 129 | ○ | 746 | 20 |
| 8137 | ⊚ | ○ | 130 | ○ | 784 | 23 |
| 8138 | ⊚ | ○ | 131 | ○ | 779 | 21 |
| 8139 | ⊚ | ○ | 128 | ○ | 710 | 22 |
| 8140 | ⊚ | ○ | 131 | ○ | 717 | 22 |

**Table 29**

| No. | machinability | | | hot workability | mechanical properties | |
|---|---|---|---|---|---|---|
| | form of chippings | condition of cut surface | cutting force (N) | 700°C deformability | tensile strength (N/mm²) | elongation (%) |
| 8141 | ⊚ | ○ | 131 | ○ | 687 | 22 |
| 8142 | ⊚ | ○ | 130 | ○ | 635 | 20 |
| 8143 | ⊚ | ○ | 129 | ○ | 710 | 23 |
| 8144 | ⊚ | ○ | 130 | ○ | 662 | 24 |
| 8145 | ⊚ | ○ | 128 | ○ | 728 | 23 |
| 8146 | ⊚ | ○ | 129 | ○ | 753 | 21 |
| 8147 | ⊚ | ○ | 130 | ○ | 709 | 24 |

**Table 30**

| No. | wear resistance |
|---|---|
| | weight loss by wear (mg/100000rot.) |
| 7001a | 1.3 |
| 7002a | 0.8 |
| 7003a | 0.9 |
| 7004a | 1.4 |
| 7005a | 1.3 |
| 7006a | 1.7 |
| 7007a | 1.8 |
| 7008a | 1.2 |
| 7009a | 0.8 |
| 7010a | 2.4 |
| 7011a | 1.9 |
| 7012a | 1.2 |
| 7013a | 1.1 |
| 7014a | 2.7 |
| 7015a | 1.4 |
| 7016a | 1.3 |
| 7017a | 1.6 |
| 7018a | 1.4 |
| 7019a | 1.9 |
| 7020a | 1.5 |

**Table 31**

| No. | wear resistance |
|---|---|
| | weight loss by wear (mg/100000rot) |
| 7021a | 1.3 |
| 7022a | 0.9 |
| 7023a | 1.2 |
| 7024a | 1.0 |
| 7025a | 2.3 |
| 7026a | 1.7 |
| 7027a | 1.8 |
| 7028a | 1.1 |
| 7029a | 1.5 |
| 7030a | 1.4 |

**Table 32**

| No. | wear resistance |
|---|---|
| | weight loss by rear (ng/100000rot.) |
| 8001a | 1.4 |
| 8002a | 1.1 |
| 8003a | 0.9 |
| 8004a | 1.2 |
| 8005a | 1.8 |
| 8006a | 1.3 |
| 8007a | 1.5 |
| 8008a | 1.0 |
| 8009a | 1.2 |
| 8010a | 0.7 |
| 8011a | 1.0 |
| 8012a | 1.3 |
| 8013a | 1.4 |
| 8014a | 1.3 |
| 8015a | 1.5 |
| 8016a | 0.9 |
| 8017a | 1.4 |
| 8018a | 0.9 |
| 8019a | 1.0 |
| 8020a | 1.5 |

**Table 33**

| No. | wear resistance |
|---|---|
| | weight loss by wear (mg/100000rot.) |
| 8021a | 1.0 |
| 8022a | 1.4 |
| 8023a | 1.4 |
| 8024a | 0.8 |
| 8025a | 1.2 |
| 8028a | 1.4 |
| 8027a | 1.9 |
| 8028a | 0.9 |
| 8029a | 1.4 |
| 8130a | 2.2 |
| 8131a | 2.1 |
| 8132a | 1.0 |
| 8133a | 2.4 |
| 8134a | 1.4 |
| 8135a | 1.2 |
| 8136a | 1.5 |
| 8137a | 1.3 |
| 8138a | 0.8 |
| 8139a | 1.4 |
| 8140a | 1.5 |

**Table 34**

| No. | wear resistance |
|---|---|
| | weight loss by wear (mg/100000rot.) |
| 8041a | 1.5 |
| 8042a | 1.3 |
| 8043a | 1.6 |
| 8044a | 1.2 |
| 8045a | 1.0 |
| 8046a | 2.0 |
| 8047a | 1.6 |
| 8048a | 1.7 |
| 8049a | 1.3 |
| 8050a | 1.5 |
| 8051a | 1.0 |
| 8052a | 1.5 |
| 8053a | 1.3 |
| 8054a | 1.2 |
| 8055a | 0.7 |
| 8056a | 0.9 |
| 8057a | 1.6 |
| 8058a | 2.4 |
| 8059a | 1.6 |
| 8060a | 1.9 |

**Table 35**

| No. | wear resistance |
|---|---|
| | weight loss by wear (mg/100000rot.) |
| 8061a | 1.6 |
| 8062a | 1.9 |
| 8063a | 1.2 |
| 8064a | 1.7 |
| 8065a | 2.0 |
| 8068a | 1.4 |
| 8067a | 1.5 |
| 8068a | 1.2 |
| 8069a | 0.9 |
| 8070a | 1.0 |
| 8071a | 1.7 |
| 8072a | 1.9 |
| 8073a | 1.6 |
| 8014a | 1.6 |
| 8075a | 1.8 |
| 8076a | 0.8 |
| 8077a | 1.3 |
| 8078a | 1.2 |
| 8079a | 1.4 |
| 8080a | 1.3 |

**Table 36**

| No. | wear resistance |
|---|---|
| | weight loss by wear (mg/100000rot) |
| 8081a | 1.6 |
| 8082a | 1.3 |
| 8083a | 1.0 |
| 8084a | 1.2 |
| 8085a | 1.5 |
| 8086a | 1.6 |
| 8087a | 1.1 |
| 8088a | 2.0 |
| 8089a | 1.4 |
| 8090a | 1.2 |
| 8091a | 1.5 |
| 8092a | 1.6 |
| 8093a | 2.1 |
| 8094a | 1.5 |
| 8095a | 1.9 |
| 8096a | 1.5 |
| 8097a | 1.5 |
| 8098a | 1.4 |
| 8099a | 1.1 |
| 8100a | 0.9 |

**Table 37**

| No. | wear resistance |
|---|---|
| | weight loss by wear (mg/100000rot.) |
| 8101 | 1.4 |
| 8102 | 1.3 |
| 8103 | 0.8 |
| 8104 | 0.8 |
| 8105 | 0.7 |
| 8106 | 0.9 |
| 8107 | 1.2 |
| 8108 | 1.1 |
| 8109 | 1.0 |
| 8110 | 0.7 |
| 8111 | 0.8 |
| 8112 | 1.2 |
| 8113 | 0.9 |
| 8114 | 1.2 |
| 8115 | 1.1 |
| 8116 | 1.4 |
| 8117 | 1.1 |
| 8118 | 0.9 |
| 8119 | 1. |
| 8120 | 0.9 |

**Table 38**

| No. | wear resistance |
|---|---|
| | weight loss by wear (mg/100000rot.) |
| 8121a | 1.0 |
| 8122a | 1.0 |
| 8123a | 1.2 |
| 8124a | 0.8 |
| 8125a | 1.1 |
| 8126a | 0.9 |
| 8127a | 1.3 |
| 8128a | 1.4 |
| 8129a | 1.3 |
| 8130a | 1.5 |
| 8131a | 1.2 |
| 8132a | 1.3 |
| 8133a | 0.8 |
| 8134a | 1.0 |
| 8135a | 0.8 |
| 8136a | 1.3 |
| 8137a | 1.1 |
| 8138a | 0.9 |
| 8139a | 1.2 |
| 8140a | 1.0 |

**Table 39**

| No. | wear resistance |
|---|---|
| | weight loss by wear (ng/100000rot ) |
| 8141a | 1.4 |
| 8142a | 1.8 |
| 8143a | 1.6 |
| 8144a | 1.9 |
| 8145a | 1.1 |
| 8146a | 1.2 |
| 8147a | 1.4 |

**Table 40**

| No. | rear resistance |
|---|---|
| | weight loss by wear (ng/100000rot.) |
| 14001a | 500 |
| 14002a | 620 |
| 14003a | 520 |
| 14004a | 450 |
| 14005a | 25 |
| 14006a | 600 |

## Claims

1. A lead-free, free cutting copper alloy which comprises 62 to 78 percent, by weight, of copper; 2.5 to 4.5 percent, by weight, of silicon; at least one element selected from among 0.3 to 3.0 percent, by weight, of tin, 0.2 to 2.5 percent, by weight, aluminium, and 0.02 to 0.25 percent, by weight, of phosphorous; at least one element selected from among 0.7 to 3.5 percent, by weight, manganese, and 0.7 to 3.5 percent, by weight, nickel; optionally at least one element selected from among 0.02 to 0.4 percent, by weight, of bismuth, 0.02 to 0.4 percent, by weight, of tellurium and 0.02 to 0.4 percent, by weight, selenium; and the remaining percent, by weight, of zinc and wherein the metal structure of the free cutting copper alloy has at least one phase selected from the γ (gamma) phase and the κ (kappa) phase.

2. A lead free, free-cutting copper alloy according to claim 1 wherein when cut on a circumferential surface by a lathe provided with a point nose straight tool at a rake angle of -8 (minus 8) and at a cutting rate of 50m/min, a cutting depth of 1.5 mm, a feed rate of 0.11 min/rev yields a chips having one or more shapes selected from the group consisting of an arch shape and a fine needle shape.

3. A lead free, free-cutting copper alloy according to any one of the preceding claims which is subjected to a heat treatment for 30 minutes to 5 hours at 400 to 600°C.

4. A method of forming a lead-free, free cutting alloy having a metal structure which has at least one phase selected from the γ (gamma) phase and the κ (kappa) phase which comprises alloying copper and silicon in an amount of 62 to 78 percent, by weight, of copper; 2.5 to 4.5 percent, by weight, of silicon; at least one element selected from tin, aluminium and phosphorous in an amount of 0.3 to 3.0 percent, by weight, of tin, 0.2 to 2.5 percent, by weight, of aluminium and 0.02 to 0.25 percent, by weight, of phosphorous; at least one element selected from manganese and nickel in an amount of 0.7 to 3.5 percent, by weight, of manganese and 0.7 to 3.5 percent, by weight, of nickel; optionally at least one element selected from bismuth, tellurium and selenium in an amount of 0.02 to 0.4 percent, by weight, of bismuth, 0.02 to 0.4 percent, by weight, of tellurium and 0.02 to 0.4 percent, by weight, of selenium; and the remaining percent, by weight, of zinc.

5. The method of claim 4 wherein said silicon is provided as a Cu-Si alloy.

6. The method of any one of claims 4 to 5 wherein said lead-free, free cutting alloy is subjected to a heat treatment for 30 minutes to 5 hours at 400 to 600°C.

## Patentansprüche

1. Bleifreie, schnittige Kupferlegierung, enthaltend:
62 bis 78 Gew.-% Kupfer, 2,5 bis 4,5 Gew.-% Silizium; wenigstens ein Element ausgewählt aus [der Gruppe] 0,3 bis 3,0 Gew.-% Zinn, 0,2 bis 2,5 Gew.-% Aluminium, und 0,02 bis 0,25 Gew.-% Phosphor;
wenigstens ein Element ausgewählt aus [der Gruppe] 0,7 bis 3,5 Gew.-% Mangan und 0,7 bis 3,5 Gew.-% Nickel; optional wenigstens ein Element ausgewählt aus [der Gruppe] 0,02 bis 0,4 Gew.-% Bismut, 0,02 bis 0,4 Gew.-% Tellur und 0,02 bis 0,4 Gew.-% Selen;
wobei der restliche Gew.-%-Gehalt Zink ist und worin die Metall-Struktur der schnittigen Kupferlegierung wenigstens eine Phase gewählt aus γ(gamma)-Phase und κ(kappa)-Phase besitzt.

2. Bleifreie, schnittige Kupferlegierung nach Anspruch 1, wobei dann, wenn diese auf einer ringförmigen Oberfläche mit einer Drehmaschine, die mit einem geraden Drehspitzmeißel ausgestattet ist, mit einem Spanwinkel von -8 (minus 8) und einer Zerspangeschwindigkeit von 50m/min, einer Schneidtiefe von 1,5 mm, einem Vorschub von 0,11 min/Umdrehung spanabhebend bearbeitet wird, Späne ergibt, die eine oder mehrere Formen ausgewählt aus der Gruppe Bogenform oder feine Nadelform haben.

3. Bleifreie, schnittige Kupferlegierung nach einem der vorhergehenden Ansprüche, die einer Wärmebehandlung von 30 Minuten bis 5 Stunden bei 400 bis 600° C ausgesetzt wird.

4. Verfahren zur Herstellung einer bleifreien, schnittigen Kupferlegierung, die eine Metall-Struktur hat, die wenigstens eine Phase, gewählt aus γ(gamma)-Phase und k(kappa)-Phase besitzt, wobei das Verfahren das Legieren von Kupfer und Silizium in einer Menge von 62 bis 78 Gew.-% Kupfer; 2,5 bis 4,5 Gew.-% Silizium umfasst;
sowie von wenigstens einem Element ausgewählt aus Zinn, Aluminium und Phosphor in einer Menge von 0,3 bis 3,0 Gew.-% Zinn, 0,2 bis 2,5 Gew.-% Aluminium und 0,02 bis 0,25 Gew.-% Phosphor;
von wenigstens einem Element ausgewählt aus Mangan und Nickel in einer Menge von 0,7 bis 3,5 Gew.-% Mangan, und 0,7 bis 3,5 Gew.-% Nickel;
optional von wenigstens einem Element ausgewählt aus Bismut, Tellur und Selen in einer Menge von 0,02 bis 0,4 Gew.-% Bismut, 0,02 bis 0,4 Gew.-% Tellur und 0,02 bis 0,4 Gew.-% Selen; wobei der restliche Gew.-%-Gehalt Zink ist.

5. Verfahren nach Anspruch 4, wobei das Silizium als eine Cu-Si-Legierung beigefügt wird.

6. Verfahren nach einem der Ansprüche 4 oder 5, wobei die genannte bleifreie, schnittige Legierung einer Wärmebehandlung von 30 Minuten bis 5 Stunden bei 400 bis 600° C ausgesetzt wird.

## Revendications

1. Alliage de cuivre de décolletage sans plomb qui comprend 62 à 78 pour cent, en poids, de cuivre ; 2,5 à 4,5 pour cent, en poids, de silicium ; au moins un élément choisi parmi 0,3 à 3,0 pour cent, en poids, d'étain, 0,2 à 2,5 pour cent, en poids, d'aluminium et 0,02 à 0,25 pour cent, en poids, de phosphore ; au moins un élément choisi parmi 0,7 à 3,5 pour cent, en poids, de manganèse et 0,7 à 3,5 pour cent, en poids, de nickel ; facultativement au moins un élément choisi parmi 0,02 à 0,4 pour cent, en poids, de bismuth, 0,02 à 0,4 pour cent, en poids, de tellure et 0,02 à 0,4 pour cent, en poids, de sélénium ; et le pourcentage restant, en poids, de zinc et dans lequel la structure métallique de l'alliage de cuivre de décolletage comporte au moins une phase choisie parmi la phase γ(gamma) et la phase κ(kappa).

2. Alliage de cuivre de décolletage sans plomb selon la revendication 1, qui, lorsqu'il est découpé sur une surface circonférentielle par un tour muni d'un outil droit à nez en pointe selon un angle de coupe de -8 (moins 8) et à une vitesse de coupe de 50 m/min, une profondeur de coupe de 1,5 mm, une vitesse d'alimentation de 0,11 min/tour, donne des copeaux ayant une ou plusieurs formes choisies dans le groupe constitué par une forme en arcade et une forme en aiguille fine.

3. Alliage de cuivre de décolletage sans plomb selon l'une quelconque des revendications précédentes, qui est soumis à un traitement de chaleur pendant 30 minutes à 5 heures à 400 à 600 °C.

4. Procédé de formation d'un alliage de décolletage sans plomb présentant une structure métallique qui comporte au moins une phase choisie parmi la phase γ(gamma) et la phase κ(kappa) qui comprend la formation d'un alliage de cuivre et de silicium à une quantité de 62 à 78 pour cent, en poids, de cuivre ; 2,5 à 4,5 pour cent, en poids, de silicium ; au moins un élément choisi parmi l'étain, l'aluminium et le phosphore à une quantité de 0,3 à 3,0 pour cent, en poids, d'étain, 0,2 à 2,5 pour cent, en poids, d'aluminium et 0,02 à 0,25 pour cent, en poids, de phosphore ; au moins un élément choisi parmi le manganèse et le nickel à une quantité de 0,7 à 3,5 pour cent, en poids, de manganèse et 0,7 à 3,5 pour cent, en poids, de nickel ; facultativement au moins un élément choisi parmi le bismuth, le tellure et le sélénium à une quantité de 0,02 à 0,4 pour cent, en poids, de bismuth, 0,02 à 0,4 pour cent, en poids, de tellure et 0,02 à 0,4 pour cent, en poids, de sélénium ; et le pourcentage restant, en poids, de zinc.

5. Procédé selon la revendication 4, dans lequel ledit silicium est fourni sous la forme d'un alliage de Cu-Si.

6. Procédé selon l'une quelconque des revendications 4 à 5, dans lequel ledit alliage de décolletage sans plomb est soumis à un traitement de chaleur pendant 30 minutes à 5 heures à 400 à 600 °C.
